

# United States Patent

[15] 3,696,128

[45] Oct. 3, 1972

[54] PERFLUOROPOLYETHER ESTERS OF QUINONES

[72] Inventor: **Bruce Hollis Garth, Newark, Del.**

[73] Assignee: **E. I. du Pont de Nemours and Company, Wilmington, Del.**

[22] Filed: June 8, 1970

[21] Appl. No.: 44,649

[52] U.S. Cl. .... 260/376, 252/54.6, 260/368,  
260/396 R

[51] Int. Cl..... C07c 69/66  
[58] Field of Search..... 260/376, 396 R, 368, 535

[56] References Cited

## UNITED STATES PATENTS

|           |        |                   |         |
|-----------|--------|-------------------|---------|
| 3,250,807 | 5/1966 | Fritz et al. .... | 260/535 |
| 3,250,808 | 5/1966 | Moore et al. .... | 260/535 |
| 3,250,806 | 5/1966 | Warnell.....      | 260/535 |

*Primary Examiner*—Lorraine A. Weinberger

*Assistant Examiner*—E. Jane Skelly

*Attorney—Nicholas J. Masington, Jr.*

[57] ABSTRACT

## Perfluoropolyether esters of quinones having the formula



wherein R<sub>1</sub> is a perfluoroalkyl group having from one to six carbon atoms, m is an integer of from 1 to 3, n is from 0 to about 20, R'<sub>1</sub> is a perfluoroalkylene group having from two to 10 carbon atoms, V is F or CF<sub>3</sub>, Q is a quinone radical and p is the number of hydroxyl groups on Q which are esterified; and fluorinated oils containing these esters.

**10 Claims, No Drawings**

## PERFLUOROPOLYETHER ESTERS OF QUINONES

## BACKGROUND OF THE INVENTION

## 1. Field of the Invention

This invention relates to novel perfluoropolyether esters of hydroxy quinones which are useful as stabilizers in fluorinated oils to reduce degradation of these fluorinated oils at high temperatures, e.g., 260° to 370°C., when the oils are used as lubricating oils, e.g., for aircraft turbine engines.

## 2. Description of the Prior Art

Fritz et al. in U.S. Pat. No. 3,250,807 and Moore et al. in U.S. Pat. No. 3,250,808 disclose that perfluoropolyether esters of aliphatic as well as aromatic alcohols can be made by reacting a perfluoropolyether acyl fluoride with the appropriate alcohol. Moore et al. also disclose broadly that such esters are useful as heat transfer media and solvents. Neither reference, however, discloses or suggests that such esters manifest any utility as high-temperature stabilizers for fluorinated oils.

There is at the present time a recognized need for lubricant oils which can function at temperatures above about 260°C. for extended periods of time, e.g., as turbine engine lubricants. Few oils are known, however, which approach serviceability under such conditions; among these are certain fluorinated oils, for example, oils prepared by fractionation of polymers which are chains of repeating units, e.g.,  $-(C_3F_6O)-$ , 30 which chains are suitably end-capped by very stable end groups, for example, by hydrogen or, preferably, perfluoroalkoxy or perfluoroalkyl groups.

In the absence of oxygen and certain metals, such oils can function at temperatures approaching 400° to 35 425°C. At operating temperatures up to about 204°C. even when metals are present such metals do not appear to promote degradation of the oils. However, at temperatures between about 260° and 370°C. oil degradation has been found to occur, especially in the presence of alloys and metals such as steels, titanium and titanium alloys and in the presence of oxygen.

It is therefore desirable to provide these oils with an additive which eliminates or reduces oil degradation, especially at very high temperatures. The esters of the 45 present invention are effective stabilizers for fluorinated oil.

## SUMMARY OF THE INVENTION

Perfluoropolyether esters of quinones having the formula



wherein  $R_f$  is a perfluoroalkyl group having from one to six carbon atoms,  $m$  is an integer of from one to three,  $n$  is from 0 to about 20,  $R'$  is a perfluoroalkylene group having from two to 10 carbon atoms,  $V$  is F or  $CF_3$ ,  $Q$  is a quinone radical having from 10 to 14 carbon atoms and  $p$  is the number of hydroxyl groups on  $Q$  which are esterified and may be from one to three.

## DESCRIPTION OF THE INVENTION

The compositions of the present invention include 20 perfluoropolyether acyl esters of hydroxy quinones, said hydroxy quinones having from 10 to 14 carbon atoms and from one to three hydroxyl groups. Representative of such esters are those having the formulas





and the like.

The esters of this invention are immiscible in water. In addition to their utility as stabilizers for fluorinated oils at high temperatures, they may also be used to lubricate machine parts, e.g., gears.

Preferred because of their effectiveness as high-temperature stabilizers for fluorinated oils and their ease of preparation are monoesters of 1 or 2-naphthoquinone-5,8 and diesters of 1,5-anthraquinone-9,10, wherein each ester group has the structure  $R_1O(C_{m-2m}O)_nCF(V)COO-$ , where  $R_1$ ,  $m$ ,  $n$  and  $V$  are as described above. Particularly preferred within this group are the 1,5-diesters of anthraquinone-9,10 wherein each ester group has the formula  $CF_3CF_2CF_2O-[CF(CF_3)CF_2]_n-CF(C_3)COO-$ ,  $n$  again being from 0 to about 20. It should be noted that in preparing the esters of this invention the value of  $n$  will normally be an average value since the ester product will normally contain mixtures of ester groups which vary only in their respective  $n$  values, each  $n$  value, however, being from 0 to about 20. Substantially pure esters may, however, be obtained by utilizing substantially pure acyl fluoride starting materials. These substantially pure acyl fluorides may be prepared, for example, by preparative gas chromatography of, e.g., the mixtures produced by the action of ultraviolet radiation on hexafluoropropylene in the presence of oxygen, as taught in French Patent 1,434,537.

The esters of this invention may be readily prepared by contacting a selected hydroxy or polyhydroxy quinone with the perfluoropolyether acyl fluoride which is appropriate to make the desired ester. Usually the reaction is carried out in the presence of a reagent, such as pyridine or some other tertiary amine, which acts to neutralize the by-product HF. Preferably the reaction is conducted under dry conditions, i.e., in the absence of

sufficient moisture to destroy important amounts of the water-reactive acyl fluoride.

Suitable equipment for the reaction would be obvious to one skilled in the art and could be constructed from materials such as glass or stainless steel or other non-corrosive materials. For large-scale production, a

35 glass-lined, agitable vessel having heating, cooling and reflux means is quite practical, e.g., a kettle, while on a small-scale the reaction is usually carried out in such equipment as a round bottom glass laboratory flask equipped with a condenser and a thermometer.

Generally, the reaction is carried out in such a vessel by mixing together and heating in the vessel the hydroxy or polyhydroxy quinone with at least 1 mole of 40 perfluoropolyether acyl fluoride per mol of quinone for each quinone hydroxyl group to be esterified. The specific temperature of the reaction is not critical but must be sufficient to effect the reaction between the acyl fluoride and the hydroxy quinone. Likewise, the 45 time of the reaction while not specifically critical must be sufficient to insure substantial completion of the reaction. Typical reaction times and temperatures are from about 10 to about 30 hours and from about 120°C. to about 150°C. for the diesters of anthraquinone and from about 10 to about 20 hours at about 40°C. to about 60°C. for the monoesters of the naphthoquinones.

50 The pressure employed is not critical, and ordinarily ambient atmospheric pressure is used.

The ester product can be isolated from the reaction mass by ordinary purification techniques, e.g., by 55 vacuum stripping to remove any excess acyl fluoride followed by water washing to remove amine salt. The ester material can then be dried (e.g., by vacuum stripping, heating, or by contact with a dehydrating agent). The material can also be washed, e.g., with dilute sodium or potassium carbonate or bicarbonate and then with water and dried or it may be washed with 60 water alone.

A low-boiling, inert solvent for the reaction product may be employed to facilitate separation of the ester product from the reaction mass. Such media include

ethers, such as diethylether, tetrahydrofuran, lower di-alkyl ethers of lower polyalkylene glycols, and chlorofluoroalkanes such as trichlorotrifluoroethane.

The product ester is most readily identified by means of infrared analysis. The quinone nucleus and the carbonyl group of the perfluoropolyether acyl portion of the ester having characteristic absorptions; minimization of aromatic hydroxyl absorption in the spectrogram of the finished product demonstrates degree of esterification of the quinone.

The aryl fluorides of the present invention are selected from those having the formulas



wherein  $R_1$  is a perfluoroalkyl group having from one to six carbon atoms,  $m$  is an integer of from 0 to 3,  $n$  is from 0 to about 20,  $R'$  is a perfluoroalkylene group having from two to six carbon atoms and  $V$  is H or  $CF_3$ .

The monoacyl fluorides which may be used are known in the art and can be prepared, for example by polymerizing tetrafluoroethylene oxide or hexafluoropropylene oxide either alone or in the presence of a carbonyl fluoride, a perfluoroketone or perfluoroalkanoyl fluoride as for example, in U.S. Pat. Nos. 3,250,806, 3,250,808 and 3,274,239. Alternatively, monoacyl fluorides can be prepared by the action of ultraviolet radiation on hexafluoropropylene in the presence of oxygen followed by treatment to reduce the peroxide content of the perfluoroacyl fluoride, as taught, for example, in "Chimica e L' Industria," volume 50, pp. 206 to 214 (1968).

The diacyl fluorides are also art-known and can be prepared, for example by reacting tetrafluoroethylene oxide or hexafluoropropylene oxide with the diacyl fluoride of a perfluorinated dibasic aliphatic acid having 2 to 10 carbons, as taught, for example in U.S. Pat. Nos. 3,250,806 and 3,250,807. Alternatively, the diacyl fluorides may be fractionated from mixtures produced by the action of ultraviolet radiation on hexafluoropropylene in the presence of oxygen, as taught, for example in French Patent 1,434,537.

The hydroxy quinones utilized as starting materials in the present invention have from 10 to 14 carbon atoms and from one to three hydroxyl groups each. They may be prepared by any art-known process, e.g., naphthaquinone — by the oxidation of e.g. 1,6-dihydroxy naphthalene; monohydroxy anthraquinone — by the condensation of phenol and phthalic anhydride; dihydroxy anthraquinone — by heating metahydroxy benzoic acid together with sulfuric acid; phenanthrene — by the hydrolysis of the corresponding diazotized diamino compounds; and trihydroxy anthraquinone by heating the corresponding dihydroxy compound together with a concentrated alkali.

As has been stated previously, the esters of this invention are useful as additives for fluorinated oils (lubricating oils) serving to stabilize the oils and retard their degradation when said oils are used at high temperatures, e.g., above about 260°C. and particularly between about 260° and 370°C., e.g., as lubricating oils for turbine engines, and when the oils are in contact with metals such as steels, titanium or titanium alloys and oxygen.

The base oils to which the esters of this invention may be added are fluorinated oils preferably having the structures

- a.  $X R''/O(C_m F_{2m} O)_{z+p} R'''_1 Y$  and
- b.  $[X R''/O(C_m F_{2m} O)_{z+p}]_2 R'''_1 F$

wherein  $-C_m F_{2m} O-$  is  $-CF_2O-$ ,  $-CF(CF_3)O-$ ,  $-CF_2CF_2O-$ ,  $-CF(CF_3)CF_2O-$  or  $-CF_2CF(CF_3)O-$ ,  $R'''_1$  is a perfluoroalkylene group having from one to six carbon atoms,  $R'''_1$  is the same or a different perfluoroalkylene group having from one to six carbon atoms,  $X$  is H, F or  $CF_3O-$ ,  $Y$  is H or F and may be the same as or different from  $X$  when  $X$  is H or F,  $m$  is an integer from 1 to 3,  $z$  is an integer designating the number of  $-(C_m F_{2m} O)-$  groups present in the molecule wherein  $m$  is 3,  $p$  is an integer designating the number of  $-(C_m F_{2m} O)-$  groups present in the molecule wherein  $m$  is 1 or 2 and the sum of  $z+p$  is an integer of from 0 to about 100 and  $R'''_1$  is a 1,2-perfluoroalkylene group having from two to four carbon atoms.

Representative of the structure (a) oils are:



and



Representative of the structure (b) oils, which are polyethers, is:



Those polyethers having perfluoroalkyl end groups, i.e., without C—H bonds, are usually preferred for the additive containing oils of this invention.

The more preferred base oils within the class described above have

1. a maximum volatility of 50 percent by weight at 204.4°C., as determined by Federal Test Method FTMS-791, Method 351; and
2. a maximum pour point of 10°C., as determined by ASTM-D-97.

The base oils utilized in the preferred additive containing oils of this invention should have a maximum volatility of 50 percent at 204.4°C. and a maximum pour point of 10°C. and it may be necessary to fractionate some of the oils given above to provide them with the preferred volatility and pour point. Within this classification it has been found that the fluorinated polyether oils having molecular weights of 3,000 to 13,000 are preferable. Of course, the polymerization methods used in preparing the oils give mixtures of

products so that the molecular weights are an average. Although a pure product having a specific molecular weight can be used, mixtures of products are equally useful if the variation in molecular weight is not too large. Usually, the most volatile lower molecular weight materials are removed from oils before use.

Oils having volatilities greater than 50 percent at 204.4°C. while not preferred, may be utilized in preparing the greases of this invention. Oils having pour points greater than 10°C., while not preferred, may also be used.

The esters are used in an effective amount in the fluorinated oils, by "effective amount" is meant the amount required to produce useful inhibition of oil degradation. Thus, the effective amount of additive, i.e., ester, will vary with the service intended and with the particular metals with which the oils will come in contact.

In general the amount of an ester required will be in the range of from about 0.5 percent by weight to about 5 percent by weight based on the weight of the fluorinated base oil. Additive concentrations above about 5 percent may, of course, be employed but they may produce little increase in degradation retardation effectiveness. For a general purpose, high-temperature oil it is usually preferable to add between about 1 and about 5 percent by weight of the esters. This range provides for the vast majority of the needs for the oils.

Preparation of the perfluorinated polyether oils containing the esters is by mixing of the two components in the indicated proportions for a time and at a temperature sufficient to assure solubility of the ester in the fluorinated oil. The lower molecular weight esters, for example, where  $n$  is from 0 to about 4 are best mixed with the oils at about 100°C. to assure complete solubility. The solubility of the esters wherein  $n$  is greater than about 5 is usually essentially complete at between 25° and 100°C., while the esters with  $n$  equal to 10 to 20 are usually completely soluble at room temperature, i.e., at about 20° to 25°C.

Fluorinated oils stabilized with the esters of the invention have practical advantages over such oils unstabilized. For example, at the high temperatures met in modern aircraft turbine engines where such oils, when used as lubricants, contact steel and titanium alloy components, the stabilized oils resist viscosity degradation and the closely associated volatilization of the lubricant oil. Lubricant loss is minimized. Periods between oil replacement are extended. Higher operating temperatures may be employed and engine heat efficiency thereby improved.

#### EXAMPLES

The following examples are intended to be merely illustrative of the invention and not in limitation thereof. Unless otherwise indicated, all quantities are by weight.

#### EXAMPLE 1

A mixture of 24 parts (0.1 mole) of 1,5-dihydroxyanthraquinone 170 parts (0.3 mole) of  $\text{CF}_3\text{CF}_2\text{CF}_2\text{OCF}(\text{CF}_3)\text{CF}_2\text{OCF}(\text{CF}_3)\text{COF}$  and 18 parts of pyridine (0.2 mole) were refluxed for 16 hours at about 120° to 140°C. in a round bottom glass laboratory flask equipped with a condenser and a thermometer. The resulting reaction mass was then subjected to a water pump vacuum stripping at 115°C. until substantially all

distillation stopped. The stripped mixture was suspended in about 400 parts of trichlorotrifluoroethane. The suspension was washed with 5 percent aqueous  $\text{NaHCO}_3$  and with 5 percent aqueous hydrochloric acid. After drying the resultant trichlorotrifluoroethane solution over anhydrous  $\text{MgSO}_4$ , the solution was freed of most of the solvent by vacuum stripping at 100°C. A semi-solid product resulted. An 8 part portion by weight of the semi-solid was heated for about 16 hours at 140°C. to complete the solvent evaporation.

The resulting semi-solid, 6 parts by weight, was shown by infrared analysis to be substantially free of aromatic hydroxyl groups and to have the ester carbonyl absorption expected for the 1,5-dihydroxyanthraquinone diester.

The diester was found to be miscible up to about 10 percent by weight in a perfluorinated polyether oil having the formula  $\text{CF}_3\text{CF}_2\text{CF}_2\text{O}[\text{CF}(\text{CF}_3)\text{CF}_2\text{O}]_n\text{CF}(\text{CF}_3)\text{COF}$ , wherein  $n$  had an average value of about 32 and the oil having an average molecular weight of 5,800.

#### EXAMPLE 2

25 A mixture of 10 parts (0.04 mole) of 1,5-dihydroxyanthraquinone, 190 parts (0.1 mole) of  $\text{CF}_3\text{CF}_2\text{CF}_2\text{O}[\text{CF}(\text{CF}_3)\text{CF}_2\text{O}]_n\text{CF}(\text{CF}_3)\text{COF}$ , wherein  $n$  had an average value of 10, and 8 parts (0.1 mole) of pyridine was heated at 150°C. for 16 hours. The reaction mixture was then suspended in 200 parts of trichlorotrifluoroethane and the suspension was washed with distilled water. The trichlorotrifluoroethane was evaporated and 88 parts of a dark-colored oil were recovered and identified by infrared analysis as the diester of 1,5-anthraquinone-9,10.

The oil was miscible in all proportions at 25°C. in the perfluoropolyether oil of Example 1.

#### EXAMPLES 3 and 4

The same process as in Example 2 was used to prepare homologous 1,5-diesters of anthraquinone wherein  $n$  averaged 4 to 8 except that the corresponding acyl fluoride homologues were utilized in place of  $\text{CF}_3\text{CF}_2\text{CF}_2\text{O}[\text{CF}(\text{CF}_3)\text{CF}_2\text{O}]_n\text{CF}(\text{CF}_3)\text{COF}$  wherein  $n$  averaged 10. The products were both oils at room temperature and miscible in all properties in the perfluoropolyether oil of Example 1 at 100°C.

#### EXAMPLE 5

A suspension of 100 parts (0.04 mole) of the acyl fluoride  $\text{CF}_3\text{CF}_2\text{CF}_2\text{O}[\text{CF}(\text{CF}_3)\text{CF}_2\text{O}]_n\text{CF}(\text{CF}_3)\text{COF}$ ,  $n$  averaging 14, 7 parts (0.04 mole) of 2-hydroxynaphthoquinone and 10 parts of pyridine in 80 parts of trichlorotrifluoroethane were refluxed for 16 hours. The resulting reaction mass was washed with water forming a trichlorotrifluoroethane solution and an aqueous layer. The heavier trichlorotrifluoroethane solution then separated from the less dense aqueous layer. The trichlorotrifluoroethane solution was dried over anhydrous  $\text{MgSO}_4$ , treated with decolorizing charcoal and filtered. Upon removal of the trichlorotrifluoroethane, an oil was recovered. Infrared analysis showed that the oil had the structure of the 2-ester of naphthoquinone. It was found to be miscible at 5 weight percent and at 25°C. in the perfluoropolyether oil of Example 1.

Examples 6 through 17, following, illustrate the effectiveness of the esters of this invention in inhibiting the high-temperature degradation of fluorinated oils in the presence of air and steels, titanium and titanium alloys.

The test procedure is an accelerated high-temperature oxidation test designed to quickly compare the serviceability of lubricant oils under severe use conditions. Reduction in oil degradation by an additive in this test is reflected in a prolonged useful life for an oil in actual use, e.g., as a turbine engine lubricant.

#### EXAMPLES 6 to 15

The compositions of this invention were tested using a modified form of the apparatus specified in the WADD Microoxidation-Corrosion Test of High Temperature Fluids, Fluids and Greases Section, Aeronautical Systems, Wright-Patterson Air Force Base, replacing the specified Pyrex tube with an Inconel tube. Basically the apparatus consists of a 3.18 mm diameter Inconel tube adapted for mounting three washers outside the lower end. The 3.18 mm tube is inserted inside a 20.6 mm diameter vertical Inconel tube so that the washers are immersed in a body of oil contained in the larger tube. The larger tube, which is adapted with a condenser for recovering any oil which may be stripped from the tube, is inserted in an aluminum heating block.

Various metal washers of the compositions in Table I were tested.

TABLE I

| Metal in Washers                  | Compositions, % by weight                                   |
|-----------------------------------|-------------------------------------------------------------|
| <b>Group A (Steels)</b>           |                                                             |
| 410                               | 0.15% C, 12% Cr, 1% Mn, 1% Si; balance Fe                   |
| 440 C                             | 1.1% C, 17% Cr, 1% Mn, 1% Si, 0.75% Mo; balance Fe          |
| M-2                               | 4% Cr, 2% V, 0.3% W, 5% Mo; balance Fe                      |
| 52100                             | 1% C, 1.4% Cr, 0.3% Mn, 0.2% Si; balance Fe                 |
| 4140                              | 0.4% C, 0.9% Cr, 0.9% Mn, 0.31% Si, 0.2% Mo; balance Fe     |
| M-50                              | 0.8% C, 4% Cr, 0.25% Si, 4.5% Mo, 0.1% Ni; 1% V, balance Fe |
| <b>Group B (Ti and Ti Alloys)</b> |                                                             |
| A-70                              | Essentially Ti                                              |
| 6A1-4V                            | 6% al. 4% V; balance Ti                                     |
| 4A1-4MN                           | 4% al. 4% Mn; balance Ti                                    |

The tests consisted of placing test washers of the metals to be tested in the apparatus, adding sufficient of the oil composition to insure that the washers were covered, assembling the remaining apparatus and inserting it in the heating block. The oil was then heated to the test temperature and air was passed down through the smaller tube into the body of oil containing the washers. Test duration was 72 hours. Dry air flow rate into the oil during the test was 5 liters per hour, measured at 25°C.

Degradation in the test oils was evaluated by determining percent change in the viscosity of the test oil during the test. The results are expressed in Table II below as:

$$\% \text{ Viscosity change} = \frac{\text{cs. after test} - \text{cs. before test}}{\text{cs. before test}} \times 100$$

where  $cs$  is the kinematic viscosity, at 38°C., in centistrokes. When the sign of the percent viscosity change is negative, oil degradation is indicated. When the sign is positive, high temperature loss of volatile oil components is indicated. It will be noted in Table II that oil degradation was normally accompanied by increased fluid loss from the apparatus. Degradation of polymer chains provides fragments having greater volatility than the original polymer. The base oil used in the following examples had the formula  $\text{CF}_3\text{CF}_2\text{CF}_2\text{O}[\text{CF}(\text{CF}_3)\text{CF}_2\text{O}]_z\text{CF}_2\text{CF}_3$  wherein  $z$  had an average value of about 28 and the base oil had an average molecular weight of about 5,000.

TABLE II

| Example No. | Source of Ester Example No. | Table I Washer Metals | 72 Hours fluid loss and Viscosity Change |               |       | % fluid loss | % vis. change |
|-------------|-----------------------------|-----------------------|------------------------------------------|---------------|-------|--------------|---------------|
|             |                             |                       | wt. % addi- flu                          | % vis. change | loss  |              |               |
| 25          | 6                           | none                  | none                                     | 2.2           | -0.02 | 6.2          | -9.2          |
| 7           | 1                           | Group                 | 2.4                                      | 0.58          | +6.3  | 2.4          | +0.8          |
| 8           | 3                           | (Steels)              | 1.0                                      | 1.17          | +3.4  |              |               |
| 9           | 4 A                         |                       | 1.0                                      | 0.83          | +4.6  | 1.9          | +1.3          |
| 10          | 2                           |                       | 1.3                                      | 1.0           | 0     | 6.1          | -9.2          |
| 11          | none                        |                       | none                                     | 12.2          | -50.2 | 79.7         | -99.0         |
| 12          | 1                           |                       | 1.0                                      | 2.3           | +9.3  |              |               |
| 13          | 3                           | Group                 | 1.0                                      | 2.5           | +10.6 | 62.3         | -92.6         |
| 14          | 4 B                         |                       | 1.0                                      | 5.3           | -7.2  | 28.6         | -77.8         |
| 15          | 2                           | (Ti and its Alloys)   | 1.3                                      | 2.5           | +2.9  | 55.2         | -93.2         |

#### EXAMPLE 16

The test procedure and a base oil as in Examples 6 to 15 was used to evaluate the naphthoquinone ester of Example 5 at 335°C. A Ti and a Ti (6A1 4V) washer was used in the test. Without additive a -84 percent viscosity change occurred; with 5 percent of the ester the change was only -5.4 percent.

#### EXAMPLE 17

A suspension of 17 parts (0.1 mole) of 2-hydroxy-5,8-naphthoquinone, 35 parts (0.025 mole) of  $[\text{FOCCF}(\text{CF}_3)[\text{OCF}_2\text{CF}(\text{CF}_3)]_n\text{OCF}_2]_2$  wherein  $n$  had an average value of 3, which is prepared from oxalyl fluoride and hexafluoropropylene oxide by the process of Example III of U.S. Pat. No. 3,250,807, 200 parts of trichlorotrifluoroethane and 2 parts of pyridine are refluxed for 17 hours. The resulting suspension is filtered and the clear filtrate is washed about 7 times with 200 parts portions 5 percent aqueous potassium carbonate and then twice with the same quantity of distilled water. The trichlorotrifluoroethane solution is freed of solvent by vacuum stripping at 140°C. at 40 mm Hg absolute pressure. Infrared analysis indicates that the resulting ester product has the expected structure, i.e.,



The results of Examples 6 to 17 clearly show the effectiveness of the esters of this invention in reducing the high-temperature degradation of fluorinated lubricant oils. It will be appreciated that even a modest increase in oil stability as indicated by this accelerated test can mean a significant increase in oil life under high-temperature use conditions. A significant commercial advantage is, thereby, provided in terms of longer life for relatively expensive oils.

The foregoing detailed description has been given for clarity of understanding only and no unnecessary limitations are to be understood therefrom. The invention is not limited to exact details shown and described for obvious modifications will occur to one skilled in the art. Similar results of prolongation and stabilization of the useful life of fluorinated oils can be effected by adding other esters with the scope of this invention.

The embodiments of the invention in which an exclusive property or privilege is claimed are defined as follows:

1. Perfluoropolyether esters of quinones having the formula

- a.  $[R_fO(C_mF_{2m}O)_nCF(V)COO]_pQ$ , or
- b.  $Q[OC(O)CF(V)(OC_mF_{2m})_nOR' O(C_mF_{2m}O)_nCF(V)COO]Q$ ,

wherein  $R_f$  is a perfluoroalkyl group having from one to six carbon atoms,  $m$  is 2 or 3,  $n$  is from 0 to about 20,  $R'_f$  is a perfluoroalkylene group having from two to 10 carbon atoms,  $V$  is F or  $CF_3$ ,  $Q$  is a quinone radical having from 10 to 14 carbon atoms and  $p$  is the number of hydroxyl groups on  $Q$  which are esterified and may be from 1 to 3.

2. Perfluoropolyether esters of quinones according to claim 1 having the formula



wherein  $R_f$  is a perfluoroalkyl group having from one to six carbon atoms,  $m$  is 2 or 3,  $n$  is from 0 to about 20,  $R'_f$  is perfluoroalkylene group having from 2 to 10 carbon atoms,  $V$  is F or  $CF_3$ ,  $Q$  is a quinone radical having from 10 to 14 carbon atoms and  $p$  is the number of hydroxyl groups on  $Q$  which are esterified and may be from 1 to 3.

3. Perfluoropolyether esters of quinones according to claim 1 having the formula



wherein  $R_f$  is a perfluoroalkyl group having from one to six carbon atoms,  $m$  is 2 or 3,  $n$  is from 0 to about 20,  $R'_f$  is a perfluoroalkylene group having from two to 10 carbon atoms,  $V$  is F or  $CF_3$  and  $Q$  is a quinone radical

55

60

65

having from 10 to 14 carbon atoms.

4. Perfluoropolyether esters of quinones according to claim 3 having the formula



wherein  $R_f$  is a perfluoroalkyl group having from one to six carbon atoms,  $m$  is 2 or 3,  $n$  is from 0 to about 20,  $R'_f$  is a perfluoroalkylene group having from two to 10 carbon atoms,  $V$  is F or  $CF_3$  and  $Q$  is a quinone radical having from 10 to 14 carbon atoms.

5. Perfluoropolyether esters of quinones according to claim 2 having the formula



wherein  $R_f$  is a perfluoroalkyl group having from one to six carbon atoms,  $m$  is 2 or 3,  $n$  is from 0 to about 20 and  $V$  is F or  $CF_3$ .

6. Perfluoropolyether esters of quinones according to claim 2 having the formula



wherein  $R_f$  is a perfluoroalkyl group having from one to six carbon atoms,  $m$  is 2 or 3,  $n$  is from 0 to about 20 and  $V$  is F or  $CF_3$ .

7. Perfluoropolyether esters of quinones according to claim 2 having the formula



wherein  $R_f$  is a perfluoroalkyl group having from one to six carbon atoms,  $m$  is 2 or 3,  $n$  is from 0 to about 20 and  $V$  is F or  $CF_3$ .

8. Perfluoropolyether esters of quinones according to claim 7 wherein the ester groups have the formula  $CF_3CF_2CFB2O[CF(CF_3)CF_2O]_n-CF(CF_3)COO-$  wherein  $n$  is from 0 to about 20.

9. Perfluoropolyether esters of quinones according to claim 8 wherein  $n$  averages 14.

10. Perfluoropolyether esters of quinones according to claim 8 wherein  $n$  averages 10.

\* \* \* \* \*

UNITED STATES PATENT OFFICE  
CERTIFICATE OF CORRECTION

Patent No. 3,696,128

Dated October 3, 1972

Inventor(s) BRUCE HOLLIS GARTH

It is certified that error appears in the above-identified patent and that said Letters Patent are hereby corrected as shown below:

In Column 12, line 46, Claim 8, the formula should read

$CF_3CF_2CF_2O[CF(CF_3)CF_2O]_n-CF(CF_3)COO-$

Signed and sealed this 1st day of May 1973.

(SEAL)

Attest:

EDWARD H. FLETCHER, JR.  
Attesting Officer

ROBERT GOTTSCHALK  
Commissioner of Patents